

July 11, 1933.

J. A. DE CEW

1,917,505

METHOD OF HYDRATING CELLULOSE FIBERS

Filed Nov. 23, 1929



BY

*Judson A. De Cew*  
ATTORNEY.

INVENTOR.

## UNITED STATES PATENT OFFICE

JUDSON A. DE CEW, OF MOUNT VERNON, NEW YORK, ASSIGNOR TO PROCESS ENGINEERS, INC., OF NEW YORK, N. Y., A CORPORATION OF NEW YORK

## METHOD OF HYDRATING CELLULOSE FIBERS

Application filed November 23, 1929. Serial No. 409,213.

In the refining and hydration of paper making fibers by means of Jordan engines, refiners, and machines of similar type, it is the common practice in the mills having more than one Jordan to a paper machine, to pass the pulp directly from one Jordan through another or through several similar machines. As many as eight of these machines may be set up in tandem and the stock allowed to pass through them all before it is considered ready for the paper machine.

I have invented an improved method of treating the paper stock with these machines and herewith disclose why an improved result is obtained.

When a raw unhydrated, or partially hydrated, cellulose fiber is fed into a Jordan engine or other hydrating machines, it is in much more viscous condition than when it comes from the machine, for the treatment softens the fibers so that they then flow more readily with the same amount of water and the stock appears thinner.

The stock entering the machines flows slowly and pumps with difficulty. There is, therefore, a limit to the density of stock that may enter the first machine under given conditions, which is lower than the density that would enter the second machine under similar conditions after the stock has passed first through the Jordan, refiner or hydrator.

My invention comprises removing a portion of the water from the stock after it has passed through one or more Jordans or machines of the Jordan type and then passing it through further machines, and repeating this practice until the treatment is finished. There are two main advantages in this process: one is that by constantly thickening the stock as it is being treated, the friction amongst the fibers is increased and less power is required by the machines. Another distinct advantage is the cooling of the stock. As the pulp stock gets hot the rate of hydration is decreased and the stock becomes freer, and when the stock is forced through directly connected Jordans the temperature often rises as high as 150° F., which is too hot to obtain either the best degree of hydration or the best sizing results.

By removing portions of water from the stock as it is being jordaned or similarly treated and repeating this operation in different stages, the temperature is not increased to the same extent, as the stock cools during the thickening process, which is only possible by intermittent operation.

In Figure 1 I show a pipe from a head box feeding the Jordan 10, as shown in my U. S. Patent No. 1,598,267. A portion of the water is then removed from the stock by means of a washer, drainer, or any other water-extracting device, 11.

In the next step I show the stock being pumped through the Jordan type engine 12 as described in my U. S. Patent No. 1,704,533, and then more water removed at 13 and finally,—after possibly one or more additional similar steps—the operation where the stock is washed and dewatered at 14.

Both of the above-mentioned patents contemplate treating the stock at high density but by different means, but do not disclose this principle of extracting water after a refining operation, which process will increase the efficiency obtained by either of the patented methods.

By this new process it is also quite feasible to Jordan or refine the stock first at low density in order to work very coarse stock and keep thickening it as the refining action takes place. After each step in the process the fibers come closer to each other, and the viscosity of the pulp mass is maintained so that the work done by the last Jordan is equal to that of those preceding it. If this process is not used and the stock is forced through a series of Jordans or hydrators, then the friction of the stock within the machine is constantly decreasing with each succeeding treatment.

Another application of this process is to add cooling water to the washers during the thickening operation, which washes and cools the stock. This is preferably applied in the latter operations. This washing operation can also be applied to remove impurities from the stock.

This process may be carried out in another manner, as disclosed diagrammatically in

Fig. 2. Here an ordinary beater, 15, containing a washer, 16, may be used as the thickening and washing machine, in which case the stock is passed alternately through a refiner, 5 similar to a Jordan, and a beater. The stock may be first broken in a beater and then pumped through a Jordan into another beater and this repeated until the stock is fully prepared, the beaters being used to thicken 10 or wash the stock as it becomes more fluid.

One beater and one Jordan might be used and operated by the batch method and the same process carried out by pumping the stock back into the beater. In this way the 15 same result would be obtained as beating the stock for a long time and then passing the stock through successive jordaning and thickening operations.

There are in use several types of machines 20 containing revolving discs with smooth or ribbed surfaces which are called hydrators or refiners, which all have a resemblance to the Jordan type machine. The general term for these is "refiner", although they could 25 also be described as Jordan type machines. Any of these machines could be used as a substitute for the Jordan in using my invention.

Various methods may be used to increase 30 the density of the stock between refining operations. In Fig. 1, I show a thickening device consisting of a tank which has a drainer bottom above the bottom of the tank, and by means of a controlled outlet a portion of 35 the water is drained away before the stock is pumped to the next refiner. Any other form of thickening may be used to increase the density during a break in the jordaning or hydrating process.

40 The type of hydrator may be changed during these operations; thus the stock might first be passed through a Marshall engine and later through a Jordan and finally through one of the revolving disc machines. 45 Between these operations the stock may be thickened by any de-watering process.

It is to be understood that the present disclosure is for the purpose of illustration only, and that the invention is not limited thereto. To those skilled in the art, many modifications of the invention will be readily 70 apparent, and it will also be obvious to such skilled persons that part of the method and means may be used without other parts thereof, many such combinations of the parts readily suggesting themselves. Therefore, it should be and is to be distinctly understood that for a definition of the limitations of the invention, reference must be had to the appended claims.

Having now described the invention, what 80 is claimed as new and for which Letters Patent of the United States is desired, is:

1. A method of treating cellulose fibers by a plurality of Jordan type refining machines, which comprises partially de-watering the 85 pulp after the first refining operation, and before the last refining operation.

2. A method of treating paper making fibers by means of Jordan type refining machines, which consists in increasing the density of the pulp after a previous jordaning operation has reduced its viscosity.

3. A method of preparing paper stock with a plurality of Jordan type refining machines, which consists in refining at a progressively 95 heavier consistency.

4. A method of treating paper pulp by means of a plurality of Jordan type refining machines, which consists in maintaining a practically constant viscosity of the pulp for each refining operation, by de-watering the pulp as the viscosity decreases.

5. A method of refining paper stock which consists in thickening the stock intermediate of the refining operations.

Signed at New York, in the county of New York, and State of New York, this 22nd day of November, 1929.

JUDSON A. DE CEW. 110